

808,339

## UNITED STATES PATENT OFFICE

JOHN COPE BUTTERFIELD, OF LONDON, ENGLAND.

## ROAD-MAKING.

No. 808,339.

Specification of Letters Patent.

Patented Dec. 26, 1905.

Application filed July 18, 1905. Serial No. 270,295.

106-78

*To all whom it may concern:*

Be it known that I, JOHN COPE BUTTERFIELD, a subject of the King of Great Britain and Ireland, residing at 13 Victoria street, 5 Westminster, London, S. W., England, have invented certain new and useful Improvements in and Relating to Road-Making, of which the following is a specification.

My invention relates to the making of roads,

10 foot-paths, pavements, and the like.

The object of the invention is to produce a good wearing and practically dustless and waterproof road to be made up at a small cost, using in the construction thereof any local

15 material which may be obtainable.

The invention consists in making up roads from any suitable hard materials of appropriate size, cemented together by a cement made up from finely-divided lime or other 20 material capable of forming a practically insoluble silicate which on exposure to the air shall form a cement-like material capable of indurating and binding together the bodies forming the road mixture into a hard concrete 25 mass.

The invention further consists in binding the materials forming the road by means of a cement made up of a mixture of finely-divided lime with a solution containing sodium silicate 30 and sugar or the like.

In carrying my invention into effect I take any local material available—for example, 35 gravel, ballast, limestone, slaked lime, chalk, sand, granite, slag, or the like—and crush the same by the use of a crusher, separating the larger coarse material from the finer by means of a revolving sieve. The former I use as a material to form the wearing-surface of the road, while the latter, after admixture with 40 from ten to fifty per cent. of powdered limestone or chalk, the proportion depending upon the composition and nature of the material in use, is mixed with a silicate-of-soda and sugar solution in such proportions that the rock-powder is sufficiently wetted to just cohere 45 together and is then spread to a depth of about three inches upon the foundation of the road. The larger pieces of rock, which are to form a wearing-surface, are then distributed evenly 50 upon the plastic mass and rolled in by a steam-

roller, so that the finer damp material is forced into the hollows existing between the larger stones, holding the same in a matrix, which in a short time becomes hard, forming one concrete mass.

The solution above mentioned is made by taking silicate of soda to strength of from 25° to 40° Twaddell and adding to it from one to five per cent. of sugar or molasses and is employed as above described. In some cases it is advisable to employ pitch and asphalt in addition to the limestone or chalk and the solution above described. When this is the case, the asphalt mixture is made up as follows: The pitch or asphalt is reduced to powder, 65 either by grinding or by a disintegrator, and mixed with seventy to eighty per cent. of limestone, or mixture of limestone with fine granite is added to the requisite quantity of asphalt—say from fifteen to twenty per cent. of 70 the whole mass ground together. The presence of the limestone or granite prevents in a great measure the softening of the pitch or asphalt during the grinding operation. According to another method the asphalt or pitch 75 may be melted in an iron caldron heated by a fire and the limestone-granite mixture added and stirred while hot and poured out to cool. When cold, the mixture may readily be broken up and ground to powder without 80 difficulty. The ground mixture is then mixed with the silicate-sugar solution and used as before to form the matrix in which the larger stones are held.

Having thus described my invention, what 85 I claim as new, and desire to secure by Letters Patent, is—

1. The herein-described improvement in the art of road-making, consisting in reducing suitable available material, separating the finer from the coarser material, mixing the finer material with limestone or chalk, a silicate of soda and a saccharine substance, thereby forming a substantially plastic mass, capable of setting hard, and thereafter firmly embedding the coarser material in said mass.

2. The herein-described improvement in the art of road-making, consisting in reducing suitable available material, separating the finer from the coarser material, mixing the

finer material with granulated asphalt or the  
like, lime or chalk, a silicate of soda and a  
saccharine substance, thereby forming a sub-  
stantially plastic mass, capable of setting hard,  
5 and thereafter firmly embedding the coarser  
materials in said mass, substantially as de-  
scribed.

In testimony whereof I have signed my name  
to this specification in the presence of two sub-  
scribing witnesses.

JOHN COPE BUTTERFIELD.  
Witnesses:

FRANCIS J. BIGNELL,  
BERTRAM H. MATTHEWS.